

March 21, 1939.

L. F. ROWE

2,151,233

LENS BLOCKING

Filed Jan. 21, 1937



FIG. I



FIG. II



FIG. III



FIG. IV



FIG. V

INVENTOR

LOUIS F. ROWE

BY

Harry A. Styll  
ATTORNEY

## UNITED STATES PATENT OFFICE

2,151,233

## LENS BLOCKING

Louis F. Rowe, Southbridge, Mass., assignor to  
 American Optical Company, Southbridge, Mass.,  
 a voluntary association of Massachusetts

Application January 21, 1937, Serial No. 121,608

3 Claims. (Cl. 51—216)

This invention relates to repetitive blocking of lenses or lens blanks; and has for one of its objects an improved method of blocking lenses which makes it possible to repeatedly use the same lens block.

5 A further object of the invention is to provide a block which is of such material as to be usable a large number of times without reshaping or replacement of any part of the block.

10 In the drawing that illustrates my invention Fig. I is a central sectional view of a block composed substantially entirely of the novel material;

15 Figs. II and III are similar views of blocks having inserts of the novel material; and

Figs. IV and V are respectively a sectional view and a view in side elevation of a modification of the block shown in Fig. I.

20 So far as shape and contour are concerned, the blocks disclosed in the figures of the drawing conform to conventional practice. In Fig. I the block has a body portion 4 provided with a plurality of spots 5 on which the lenses may be mounted. The body portion 4 is carried by a metal adapter 25 6 which may include anchoring means 7 and a base plate 7a. The adapter has a key slot 7b for securing the block on an actuating member, such as a spindle for rotation of the block during a surfacing operation.

30 In Fig. II the block has a metal body portion 8 with inserts 9 which take the place of the spots 5 on the form of block shown in Fig. I. The adapter for the body portion 8 is shown at 10.

In the form of block shown in Fig. III the body 35 portion 12 is dished and carries a plurality of inserts 13 on which the lenses or lens blanks are to be mounted.

In the form of block shown in Figs. IV and V there is a metal core 15 overlaid with molded 40 material 16, the spots 5a being molded as an integral part of the latter, as indicated in Fig. IV. The metal core 15 has the usual adapter, as shown at 16.

45 According to customary practice for surfacing the second side of a lens after the first side has been already surfaced, a block is used having a core of metal of substantially the character shown at 15 in Fig. IV. To prepare for blocking, according to customary practice, this core is overlaid with pitch, the spots on the pitch being each molded to approximately the required shape of the side of the lens which has already been surfaced. In the process of actually blocking the lenses, the spots are sufficiently softened by heat 50 to conform to the lens surfaces applied thereto.

According to my invention I deviate from the customary practice by employing a resinous material for the entire block, as in the form shown in Fig. I, or for inserts, such as shown at 9 and 13 in Figs. II and III respectively, or for the overlaid portion 16 shown in Figs. IV and V.

5 In general, the most economical is the form of my invention shown in Fig. I, in which the body portion 4 is molded of resinous material. The body portion 4 can conveniently be molded from a mix which is plastic when formed. It is optional whether the mix be a permanently hardenable one or not. Non-polymerizing resins have the advantage that the blocks may be ground up and again molded to make new blocks as desired. Resins which are permanently hardenable, such as synthetic resins of the phenol formaldehyde condensation products type, are usable with or without a filler or fillers for the body portion 4. The synthetic resins of the phenol formaldehyde type are customarily molded under heat and pressure, and under these conditions become permanently rigid and will then be substantially unaffected by heat below the charring point.

25 When such a permanently hardened resinous material is employed as the body portion 4, it is usable for blocking lenses L by first painting the spots 5 with a thin coating of an adhesive paint 7'. A block of this character is very durable so that blocking can be repeated almost indefinitely without replacement of the block becoming necessary.

30 The resinous material of the body portion 4 and of the spots 5 has a low rate of heat conductivity, so that the adhesive paint 7' readily adheres to the warm lenses during blocking. This is a distinct advantage over the use of a metal block with adhesive paint applied as a coating to the spots, since the heat from the warm lenses flows into the cold metal of the body portion of metal blocks so rapidly as to render the coating of paint substantially non-adhesive to the glass.

35 As above mentioned, the body portion 4 and the spots 5 of the block may be composed of a filler and a resinous binder which does not become permanently hardened under heat treatment. Moreover, I have found such a composition to be particularly advantageous for the inserts shown at 9 and 13 in Figs. II and III respectively. In this case the body portion 8 or 40 12 may be cast iron, or may be a composition including phenol formaldehyde synthetic resin with or without a filter, or other suitable material. It is not necessary to employ an adhesive 45 50 55

paint, since the lenses will adhere to the resinous material 9 or 13.

One composition which I have found suitable for my purpose is a mixture of 70 parts by weight of a filler, such as finely ground asbestos, and 30 parts by weight of commercial gum rosin. The relative proportions of the filler and rosin may be considerably varied.

The tackiness of the composition is increased 10 by decreasing the proportion of filler, but the material is not so rigid nor so resistant to deformation when applying the hot lenses. On the other hand, it is not desirable to reduce the proportion of rosin below 25 parts in 100, as the mix is difficult to handle. I find that a mix containing 25 parts or more of rosin in 100 produces a block sufficiently tacky. Thus increasing 15 the content of filler increases the rigidity of the resulting block.

20 Instead of the finely ground asbestos I may employ diatomaceous earth or other suitable filler. In place of commercial gum rosin I may employ synthetic resins, and more particularly non-polymerizing resins. For example, I employ chlorinated diphenyl resins and obtain a stronger 25 block or insert than when employing rosin. More particularly, I have found a good mixture to consist of 35 parts by weight of chlorinated diphenyl resin and 65 parts by weight of asbestos powder. 30 Here also the proportion of chlorinated diphenyl resin may be considerably varied; though preferably not decreased below 25 parts in 100. The filler may be the asbestos powder named, diatomaceous earth, or other suitable filler.

35 Both the mixes containing rosin and the mixes containing chlorinated diphenyl resin can be cold molded. The less tacky mixes require considerable molding pressure, and good results are obtained with hydraulic pressure. The need for 40 pressure in molding is reduced if the mix is molded hot, for instance 150° F. The hot molding results in a more solidly molded material.

45 It is notable that these mixes require no appreciable allowance for shrinkage. This is contrary to experience with pitch compounds which require an allowance of as much as  $\frac{1}{4}$  dipter on a 6 base curve. When molding these mixes, the molds are fashioned to the curve desired, and the molded block or insert retains the curve imposed by the mold.

50 An alternative method for obtaining blocks or inserts is to machine the resinous material to the desired shape.

I include within my invention the use of permanently hardenable resins and the use of non-polymerizing resins. The latter type provide spots which become tacky when hot. In mounting a hot lens or lens blank on one of the spots, I apply pressure to the hot lens or lens blank to cause it to adhere to the block. This may be repeated as often as there are spots on the block. The exposed surfaces of the lenses or lens blanks are then ground or polished, or both, after which the lenses are removed in the customary manner by chilling. The cycle is then renewed by replacing the removed lenses by hot lenses, each being applied to substantially the same position on a spot occupied by a removed lens.

70 My invention has the advantage that the spots are remarkably durable. In spite of the pressure applied when the hot lenses are mounted on the spots such as the inserts 9 and 13, these spots

are not appreciably deformed, especially if a high content of filler is employed. The adhesive characteristics of the resinous material of the non-polymerizing type are ample for firmly holding the lenses or lens blanks during grinding and 5 polishing. Resinous materials which do not provide spots which are sufficiently tacky may be painted with an adhesive paint as above suggested.

The cost of blocking is materially decreased by 10 my invention.

While I have illustrated and described certain preferred embodiments of my invention, it will be understood that the invention may be otherwise embodied and practiced within the scope of 15 the following claims.

I claim:

1. A device for supporting work pieces comprising a body portion having a preshaped attaching seat formed of a mixture of thermoplastic 20 and discrete non-thermoplastic constituents in which portions of some of said discrete particles of the non-thermoplastic constituent, throughout the seat, lie in the plane of and retain the shape of the seat and in which the thermoplastic constituent fills the voids between the discrete particles and, when subjected to heat as from a hot piece of work placed on said seat, is adapted to exude from between the discrete particles and provide means for retaining the work piece in 25 secured relation with said seat with the portion of the particles of the non-thermoplastic constituent in the plane of the seat providing a relatively positive positioning rest for said work piece.

2. A device for supporting work pieces comprising a body portion having a plurality of preshaped attaching seats thereon, the material of the portions having the preshaped attaching seats comprising a mixture of thermoplastic and discrete non-thermoplastic constituents in which 40 portions of some of said discrete particles of non-thermoplastic constituent, throughout each seat, lie in the plane of and retain the shape of said seat and in which the thermoplastic constituent fills the voids between the discrete particles and, 45 when subjected to heat as from hot pieces of work placed on said seats, is adapted to exude from between the discrete particles and provide means for retaining the work pieces in secured relation with said seats with the portions of the 50 particles of the non-thermoplastic constituent in the plane of said seats providing a relatively positive positioning rest for said work pieces.

3. A lens blank support comprising a body portion having a raised preformed attaching seat 55 thereon formed of a mixture of relatively solid particles which retain their shape under the heat of a lens and an adhesive ingredient, said preformed seat having portions of said solid particles distributed throughout the area of said seat and 60 lying in the plane of said seat with portions of the adhesive ingredient in said plane, the said adhesive having characteristics which will cause it to soften and exude from between said solid particles when subjected to heat, as from a 65 heated lens blank having a surface shaped substantially to the shape of said seat, and placed on said seat, the said adhesive, upon exusion, being adapted to adhere to the surface of the lens blank with the said surface engaging the solid 70 particles in the plane of said seat to position and hold the said lens blank on said seat.

LOUIS F. ROWE.